

## UNITED STATES PATENT OFFICE

2,600,504

FORMING PAPER FROM MODIFIED  
CALCIUM ALGINATE FIBERS

Arthur Johnson, Leeds, and Edwin George Millatt,  
Maidenhead, England, assignors to Alginate  
Industries Limited, London, England, a British  
company

No Drawing. Application June 4, 1948, Serial No.  
31,226. In Great Britain June 19, 1947

6 Claims. (Cl. 92—21)

1

This invention comprises improvements in or relating to the manufacture of paper.

Paper is ordinarily manufactured from the various forms of fibrous cellulosic materials such as wood pulp, rags, sisal fibres and the like. The fibres are beaten in water to form a pulp and the beating gives them a quality of adhesion so that when the pulp containing them is drained on a porous surface the fibres felt together and become a coherent sheet. For some purposes it would be advantageous to have soluble papers. Cellulose fibres are not soluble in water or weak acids or alkalis. Papers are made which are called "soluble" but this only means that they become so soft in water as to be readily disintegrated and to revert to the state of pulp. Paper moreover is readily inflammable and for many purposes a non-inflammable paper would be of great advantage.

It is an object of the present invention to provide paper which affords the advantages of solubility or of resistance to fire or both.

According to the present invention a process of production of paper consists in taking water-insoluble alginic fibres, comminuting them and making them into a pulp in water, rendering them adherent so as to be capable of felting together into a coherent sheet by the introduction into the pulp of a swelling agent which causes the alginic fibres to swell and become sticky in water, and then making paper from the pulp so prepared.

Water-insoluble alginic fibres do not become capable of felting when beaten in water. That is to say, although a mat of such fibres may be produced on a screen, it will not hold together when drained and dried because there is no tendency for one fibre to adhere to another. There therefore is a fundamental distinction between the process according to the present invention and the ordinary procedure of paper making, in that the fibres must be brought into a feltable condition, not by beating but by the addition to the pulp of a swelling agent.

Fibres of calcium alginate are soluble in weak alkalis such as a 1% solution of sodium carbonate. We have found however that if a sodium carbonate solution is made sufficiently weak it can be used as a swelling agent to swell the outer surface of calcium alginate fibres without dissolving the fibres, and that this combination of calcium alginate with sodium carbonate used as a swelling agent is particularly advantageous for the purpose of the present invention. Calcium alginate is also non-inflammable—that is, it does

2

not burn with a flame or propagate combustion, although it may char under heat. Consequently paper made from fibres of calcium alginate is non-inflammable and if treated with alkalis stronger than that used as a swelling agent for making the paper, it can easily be wholly dissolved therein. The invention is not however limited to the employment of calcium alginate as fibres of many other alginates such as copper alginate, zinc alginate, chromium alginate, benzylum alginate and many others which are water-insoluble have been spun. A suitable agent for any particular alginic fibre will be one which tends to dissolve the fibre but is employed in a strength sufficient only, within the time of treatment employed, to act superficially thereon so as to swell the outer layers. Agents suitable for trial for this purpose can be selected according to the known chemical properties of the alginates. For example, copper alginate is responsive to ammonium phosphate. Chromium alginate is resistant to alkalis. Not all alginates are non-inflammable, and if an inflammable alginate is employed of course the resulting paper will partake of this property. The actual strength of the swelling agent in any particular case will depend upon a number of factors including the temperature, the time of treatment and the hardness of water employed. An example of successful treatment and limits for that case are hereinafter set forth. Under other conditions a simple preliminary trial will suffice to determine the best strength to obtain the desired results.

35 The alginic fibres may be produced from known alginic yarns or staple fibres by cutting or otherwise.

By varying the concentration of alkali or other swelling agent, it is possible to control the amount of binding or adhesion which takes place between adjacent fibres, and thus to vary the characteristics of the resultant paper. The quality of the paper may also be varied by altering the length of the alginate fibres employed. In the absence of an alkali or other swelling agent there is no adhesion between the fibres of the paper and if too great a concentration of alkali is employed, the fibres become too weak and swollen to be handled conveniently.

40 50 The following example illustrates one application of the process:

*Example*

Calcium alginate fibres, consisting of waste 55 from the production of alginate staple fibres for

use in spinning yarns, were taken, chopped up fine and dispersed with tap water to form a pulp so as to produce a suspension containing 3 grams of calcium alginate fibre in each 300 millilitres of water. The water employed had a hardness of 32°, that is to say it corresponded to the presence of 32 parts of  $\text{CaCO}_3$  per 100,000 of water. 0.2 gram of sodium carbonate was added for each 300 millilitres of the above-described alginate-containing pulp, and the pulp was kept stirred at a temperature of 60-70° F. for 30 minutes. The quantity of sodium carbonate stated is sufficient to convert from 15% to 20% of the calcium alginate to sodium alginate. Sufficient of this suspension was made up to fill a shallow vat, and a sieve covered with a piece of No. 1 filter paper was immersed in the suspension so as to be filled with the pulp, removed with shaking in the usual way to cause the fibres to mat together, drained and the resulting filtered paper was transferred to a wire gauge drainer and dried thereon, and then hot-pressed to produce a strong hand-made paper sheet.

In carrying out the process by steps similar to those described in the foregoing example it has been found that 0.4 gram of sodium carbonate represents approximately the upper limit of alkali concentration for a fibre suspension consisting of 3 grams of calcium alginate fibres in 300 millilitres of water. When 0.50 gram were added the fibre became too swollen to handle and was discarded. 0.40 gram gave a parchment-like paper and smaller quantities softer and weaker papers. It is to be expected that with harder water slightly more sodium carbonate would be required. This quantity corresponds to the conversion of 50% to 55% of the calcium alginate to sodium alginate.

It should be noted that although calcium alginate fibre is a preferred starting material for the production of these alginate papers, other fibres made from alkali-soluble, but water-insoluble alginates may equally well be used. In the example described above, sodium carbonate was used as the swelling agent. In place of this compound when using calcium alginate fibres any of the water-soluble salts of the alkali metals, or ammonium, or magnesium which yield insoluble calcium salts may be used. All that is required of a swelling agent for any water insoluble alginate is that it be capable of causing partial conversion of the water-insoluble alginate to a water-soluble alginate.

We claim:

1. A process of making paper which consists in taking water-insoluble alkaline-earth alginate fibres, reducing them to the form of a short-

fibre aqueous pulp, introducing a soluble alkali salt of an anion which will form an insoluble salt with the alkaline earth in the insoluble alginate fibres, in sufficient quantity to combine with from 5% to 55% of the alkaline earth, thus causing the fibres to swell, and then causing the fibres to felt together to make paper.

2. A process of making paper which consists in taking water-insoluble alkaline-earth alginate fibres, reducing them to the form of a short-fibre aqueous pulp, introducing sodium carbonate in sufficient quantity to combine with from 15% to 55% of the alkaline earth in the alginate and thus causing the alginic fibres to swell, and then felting the fibres together to form paper.

3. A process of making paper which consists in taking calcium alginate fibres, reducing them to the form of a short-fibre aqueous pulp, introducing sodium carbonate in sufficient quantity to combine with from 15% to 55% of the calcium in the alginate and thus causing the alginic fibres to swell, and then felting the fibres together to form paper.

4. A process as claimed in claim 1, wherein the paper after being felted and drained is hot pressed.

5. A process as claimed in claim 2, wherein the paper after being felted and drained is hot pressed.

6. A process as claimed in claim 3, wherein the paper after being felted and drained is hot pressed.

ARTHUR JOHNSON.  
EDWIN GEORGE MILLATT.

#### REFERENCES CITED

The following references are of record in the file of this patent:

#### UNITED STATES PATENTS

| Number    | Name     | Date           |
|-----------|----------|----------------|
| 737,421   | Krefting | Aug. 25, 1908  |
| 1,509,035 | Thornley | Sept. 16, 1924 |
| 1,675,244 | Blombery | June 26, 1928  |

#### FOREIGN PATENTS

| Number  | Country       | Date           |
|---------|---------------|----------------|
| 316,119 | Great Britain | July 23, 1929  |
| 492,264 | Great Britain | Sept. 13, 1938 |

#### OTHER REFERENCES

Journal of the Society of Dyers and Colorists, vol. 62, page 100, (1946).  
Colloid Chemistry by Alexander, vol. VI, pages 718-722 (1946), published by Reinhold Publishing Corp., New York.